

P. C. H. WEST.  
TREATMENT OF LEAD SULFID ORES.  
APPLICATION FILED NOV. 24, 1915.  
1,225,296. Patented May 8, 1917.



Inventor:  
Percy Charles Harry West,  
By his Attorney  
Rosenbaum, Stockbridge & Borst

# UNITED STATES PATENT OFFICE.

PERCY C. H. WEST, OF LONDON, ENGLAND.

## TREATMENT OF LEAD-SULFID ORES.

1,225,296.

Specification of Letters Patent.

Patented May 8, 1917.

Application filed November 24, 1915. Serial No. 63,280.

*To all whom it may concern:*

Be it known that I, PERCY CHARLES HARRY West, a subject of the King of Great Britain, residing at London, England, have 5 invented certain new and useful Improvements in and Relating to the Treatment of Lead-Sulfid Ores, of which the following is a specification, reference being had therein to the accompanying drawing.

10 According to the known processes for obtaining basic lead sulfate, lead sulfid ores are fed on to a bed of incandescent coke whereby the lead sulfid is volatilized. The vaporized lead sulfid is then oxidized, in 15 some cases by air being drawn into the furnace for this purpose, in others, by air being admixed with the sulfid vapors in a separate chamber.

These processes have not been extensively 20 adopted although they yield results which from some points of view are satisfactory. In working them it has been found (1) that the iron compounds contained in the ore or in the coke are volatilized together with the 25 sulfid, even when such compounds are present only in small quantities; (2) that at the temperature obtaining in the furnaces there is formed a certain proportion of slag which is difficult to extract; (3) that much pig 30 lead is produced, (4) that the properties of the basic lead sulfate which is obtained are not all that is desired; and (5) the processes operate with a certain want of uniformity, owing, for example, to variations in the 35 temperature of the bed of coke as a whole or to local variations of temperature within the bed of coke.

The object of my invention is to overcome 40 as far as possible the above mentioned defects, and generally to effect improvements in the known processes for the production of basic lead sulfate from lead sulfid.

According to my invention, the lead sulfid is volatilized at a comparatively low 45 temperature for example 1000-1100° C.

Further, according to my invention, in 50 order to effect the volatilization of the lead sulfid at the desired low temperature, when employing a bed of incandescent coke, the air required to maintain combustion is aspirated through the bed of coke by means of a fan which also draws in the air required to oxidize the vapors and exhausts the fumes produced, and, in order to assist in maintaining the desired low temperature for the volatilization of the lead sulfid, a propor-

tion of combustion gases or other neutral gases, for example, carbon dioxid may be admixed with the air required for the combustion of the coke. By admixing such 60 gases with the air the employment of induced draft entirely, is of less importance.

When the formation of basic lead sulfate is carried out by the type of process in which air is drawn into the furnace above the level 65 of the coke in order to effect oxidation of the sulfid vapors, according to a further feature of my invention, the quantity of air so drawn in is preferably insufficient to oxidize the vapors completely and the final oxidation of the vapors is then effected in a separate chamber which is hereinafter referred to as a combustion chamber, in which the temperature of the flame is preferably such that the vapors glow with an orange red to 70 orange color, and is lower than the temperature at which the partial oxidation is carried out.

In order that the invention may be more clearly understood, the preferred method of 80 carrying the invention into effect will be described with reference to the plant illustrated in the accompanying drawings:—in which—

Figure 1 is a longitudinal section of a 85 plant suitable for carrying the invention into effect.

Fig. 2 is a transverse section on the line 1—1 of Fig. 1.

Fig. 3 is a transverse section on the line 90 2—2 of Fig. 1 and Fig. 4 is a section on a larger scale of the feeding device.

The galena is fed from a container  $\alpha$  by a suitable feeding device, for instance, a screw conveyer  $\alpha'$  into the hopper  $b$  within which may be arranged, as indicated in Fig. 4, smaller hoppers  $b_1$  and  $b_2$ , the hoppers thus arranged having discharge openings of successively decreasing size by which means 95 the ore is more accurately directed toward the apex of the cone  $c$ .

The galena falling on to the cone is uniformly distributed over the surface of the bed of incandescent coke  $d$  by means of which it is vaporized at a temperature of 100 about 1000° C.-1100° C. The vapors of lead sulfid thus produced meet a stream of air passing in at  $e$  by which they are partially oxidized and together they pass by way of the pipe  $f$  into the chamber  $g$  in which are provided openings  $h$  having dampers  $j$ . A further quantity of air is drawn in through

these openings and the incandescent vapors are thereby completely oxidized and partially cooled, the cooled gases passing by way of the conduit  $g'$  through the cooling chambers  $k_1$ ,  $k_2$ ,  $k_3$ ,  $k_4$  and  $k_5$  which are preferably constructed of thin metal, in order that the gases may rapidly be cooled. These coolers are of considerable height and depth in relation to their width and each of the chambers  $k_1$ ,  $k_2$ ,  $k_3$  and  $k_4$  is provided with a diaphragm parallel to the plane of Fig. 1 causing the gases as indicated by the arrows to travel downwardly from the point at which they enter the cooling chamber and upwardly to the point at which they pass out.

After passing through these cooling chambers which may be provided with openings having slides, in order that material deposited in them may be withdrawn, the gases and the solids suspended therein pass by way of the trunk  $n$  into the chamber  $o$ , the upper surface of which is provided with a plurality of holes  $p$ , having collars  $q$  to which flannel bags  $r$  are secured at one end by means of suitable clips. These flannel bags are suspended from the bars  $s$  which are so mounted in the walls of the chamber  $t$  that they may be pushed backward and forward in a longitudinal direction and thus the material deposited in the bags may be shaken down on to the floor of the chamber  $o$ , from which it may be removed by way of suitable openings, conveying apparatus being provided if desired to enable the material to be economically removed.

The gases freed from suspended solid matter pass through the bags into the chamber  $t$  from which by way of the trunk  $v$  they pass to the fan  $w$  and are discharged by the shaft  $x$ .

The air required to maintain the combustion of the coke is drawn by means of the fan  $w$  through an opening  $y$  the size of which by means of a slide  $y'$ , or the like may be varied, and thence between the firebars  $z$  through the bed of coke  $d$ .

The whole of the air required for the combustion of the coke, the oxidation of the sulfid vapors and for cooling are thus drawn through the several devices by means of one fan, whereas hitherto the air required for the combustion of the coke has been forced in through twyvers when a furnace similar to that now employed has been used. The temperature in the furnace is, by the method of supplying air now described kept very uniform and local overheating is prevented with the result that the whole process operates with remarkable regularity and yields a product of great uniformity of character.

The coke employed should be foundry or furnace coke and the depth of the bed of coke should be relatively considerable, for

instance, about 1.5 meters. The air admitted to the bed of coke should be limited in order to prevent the temperature rising unduly. The temperature of the vapors in the combustion chamber is kept within the desired limits, that is to say preferably within the limits between which they glow with an orange red or orange color, firstly by regulating the draft through the furnace or by introducing with the air a greater or less proportion of combustion gases, for example carbon dioxide; and secondly, by adjusting the slides  $j$  in order to permit of the entrance of a greater or less proportion of air which will thus produce a greater or less cooling action.

I claim:—

1. A process of treating lead sulfid ores to obtain basic lead sulfate which comprises feeding lead sulfid onto an incandescent bed of coke, partially oxidizing the vapors thus formed and then completing the oxidation of the vapors at a lower temperature.

2. A process of treating lead sulfid ores to obtain basic lead sulfate which comprises feeding powdered galena onto a deep bed of incandescent coke, volatilizing the lead sulfid at a uniformly low temperature, partially oxidizing the vapors formed and then completely oxidizing the vapors at a lower temperature.

3. A process of treating lead sulfid ores to obtain basic lead sulfate which comprises feeding the lead sulfid ore onto a deep bed of incandescent coke, volatilizing the lead sulfid at a temperature of 1000-1100° C., partially oxidizing the vapors formed and then completely oxidizing the vapors at a lower temperature.

4. A process for the treatment of lead sulfid ores comprising feeding the lead sulfid on to a bed of incandescent coke while maintaining the bed of coke at a temperature below that which injection of a gaseous mixture of the composition of air would cause it to assume.

5. A process for the treatment of lead sulfid ores comprising volatilizing the lead sulfid at a comparatively low temperature in an attenuated atmosphere and oxidizing the vapors produced.

6. A process for the treatment of lead sulfid ores comprising feeding the lead sulfid on to a bed of incandescent coke, maintaining the coke in a state of incandescence by aspirating air therethrough and oxidizing the vapors produced.

7. A process of treating lead sulfid ores to obtain basic lead sulfate which comprises feeding the powdered ore on to a bed of incandescent coke in a furnace, volatilizing the lead sulfid at a temperature of about 1000-1100° C., admitting to the furnace above the level of the coke a quantity of air insufficient to oxidize the vapors of lead

sulfid completely, causing the partially oxidized vapors to pass to a chamber, and completing the oxidation of the vapors at a lower temperature.

- 5 8. A process of treating lead sulfid ores to obtain basic lead sulfate which comprises feeding the powdered ore onto a bed of incandescent coke in a furnace, volatilizing the lead sulfid at a temperature of 1000-  
10 1100° C. admitting to the furnace above the level of the coke a quantity of air insufficient to oxidize the vapors of lead sulfid completely, passing the vapors into a chamber and further oxidizing the vapors  
15 therein at such temperature that the vapors glow with an orange-red to orange color.  
9. A process of treating lead sulfid ores to obtain basic lead sulfate which comprises aspirating air through a bed of incandescent coke in a furnace, feeding powdered galena onto a bed of coke, volatilizing the lead sulfid at a temperature of 1000-1100° C., aspirating air into the furnace above  
20 the level of the coke in a quantity insuffi-

cient to oxidize the vapors completely, aspirating the partially oxidized vapors into a chamber, admitting air to this chamber and effecting the complete oxidation of the lead sulfid.

10. Apparatus for the treatment of lead sulfid ores comprising a furnace, means for feeding the ore thereto, means for aspirating air therethrough, means for admitting air above the fuel level in the furnace means for aspirating the gaseous products therefrom, a chamber connected to said means, means for admitting air to said chamber, a plurality of cooling chambers connected thereto and means connected to the last of said cooling chambers for aspirating the solids from the gases passing therethrough.

In testimony whereof I have affixed my signature in the presence of two witnesses.

PERCY C. H. WEST.

Witnesses:

F. A. S. GWATKIN,  
FRANCIS AIRNLAND.